

# UNITED STATES PATENT OFFICE.

THOMAS ARCHIBALD GOODCHILD AND ARCHIBALD CAMPBELL TAIT BOND,  
OF LONDON, ENGLAND.

## PROCESS OF PRODUCING WATER-MARKS IN OR ON MANUFACTURED PAPER.

SPECIFICATION forming part of Letters Patent No. 625,255, dated May 16, 1899.

Application filed December 27, 1898. Serial No. 700,454. (No specimens.)

*To all whom it may concern:*

Be it known that we, THOMAS ARCHIBALD GOODCHILD and ARCHIBALD CAMPBELL TAIT BOND, subjects of the Queen of Great Britain and Ireland, residing at London, in the county of Middlesex, England, have invented a certain new and useful Process for the Production of Water-Marks in or on Manufactured Paper, of which the following is a specification.

10 Our invention relates to improvements in the production of disappearing but repeatedly-revivable water-marks in or on manufactured paper; and the object is to attain this result in a simple manner and by the application of electricity.

In putting our invention into practice we proceed as follows: Upon a platinum sheet or plate forming the anode we place a layer of absorbent material, such as blotting-paper, 20 previously moistened with water. On this material we place the paper which is to receive the water-mark, the paper having been previously moistened through with water. We then press face downward on the paper a 25 platinum design of the water-mark, and this design forms the cathode. We keep the paper in contact with the design for some five to ten seconds, according to the nature of the paper and the amount of electric current used. The result on removal of the cathode is a distinct and translucent image of the 30 design, which gradually fades as the paper dries and finally becomes invisible. The mark can, however, be revived and made visible as often 35 as the paper is immersed in water or moistened in any other manner.

In our experiments we have employed and found suitable an electric current of one ampere at ten volts.

40 We offer the following as the most probable explanation of the changes which take place in the paper, the explanation being the result of duly-verified experiments. Ordinary

drinking-water contains saline substances in solution and that used by us did so to the extent of twenty grains to the gallon. These saline substances are decomposed by the passage of the electric current, acids with oxygen being liberated at the anode and alkalies with hydrogen appearing (as  $\text{NaHO}$ , &c.) at the cathode, where it comes in contact with the paper, the result being that the paper becomes more hygroscopic at these points of contact. We have reason to believe, however, that the change is not limited to this, but that this 55 particular portion of the paper or cellulose combines with an additional molecule of water, thereby becoming one or other of the glucoses. If we consider the paper (cellulose) as  $\text{C}_6\text{H}_{10}\text{O}_5 + \text{H}_2\text{O}$ , we have  $\text{C}_6\text{H}_{12}\text{O}_6$ —a glucose 60 or some body resembling it in chemical composition. The change may be due to the nascent hydrogen.

What we claim as our invention, and desire to secure by Letters Patent, is— 65

The process herein described for producing in or on manufactured paper a disappearing but repeatedly-revivable water-mark the said mark being invisible in a dry but visible in a moistened condition of the paper, the said 70 process consisting in placing on a platinum plate or sheet forming the anode, a layer of absorbent material saturated with water, in placing on this and in a moistened state the paper which is to be watermarked and in 75 pressing face downward on the paper a salient or other platinum design forming the cathode so that the current from a source of electricity may pass through that portion of the paper which is in contact with the design on the 80 cathode.

THOMAS ARCHIBALD GOODCHILD.  
ARCHIBALD CAMPBELL TAIT BOND.

Witnesses:

H. PEATREY,  
F. ANDREWS.